

## UNITED STATES PATENT OFFICE.

GEORGE GUILLAUME ANDRÉ, OF GLENLEAN SANDBANK, NEAR GREENOCK, SCOTLAND, ASSIGNOR TO CHARLES HERBERT CURTIS, OF LONDON, ENGLAND.

## MANUFACTURE OF GUNPOWDER.

SPECIFICATION forming part of Letters Patent No. 576,532, dated February 9, 1897.

Application filed May 6, 1892. Serial No. 432,045. (No specimens.) Patented in England July 4, 1891, No. 11,383.

To all whom it may concern:

Be it known that I, GEORGE GUILLAUME ANDRÉ, civil engineer, a subject of the Queen of Great Britain, residing at Glenlean Sandbank, near Greenock, in the county of Renfrew, Scotland, have invented certain new and useful Improvements in the Manufacture of Gunpowder, (for which I have received Letters Patent in Great Britain No. 11,383, bearing date July 4, 1891;) and I do hereby declare that the following is a full, clear, and exact description of the invention, which will enable those skilled in the art to which it appertains to make and use the same.

Heretofore nitrocellulose, either in the soluble form (as dinitrocellulose) or in the insoluble form, (as trinitrocellulose,) has been used in combination with nitroglycerin as an ingredient in explosives for blasting purposes and more recently in smokeless gunpowder. It has also been proposed to make explosives consisting of nitroglycerin and trinitrocellulose with a small proportion of dinitro, (partly accidentally present and partly sometimes purposely added,) the solution and thorough combination of the ingredients being effected by heat and heavy pressure, together with a small amount of a suitable solvent, such as acetone or acetic ether, or by such solvent alone at the ordinary temperature or slightly above it. Now it has been discovered, by a series of experiments extending over a long period of time, that a compound containing about two parts by weight of trinitrocellulose, the so-called "insoluble" nitrocellulose, and one part by weight of dinitrocellulose (the so-called "soluble" nitrocellulose) forms a base which, in combination with nitroglycerin all thoroughly combined by the aid of a suitable solvent, such as acetone or acetic ether, gives a product differing materially in its physical qualities from those obtained from the use of mainly one variety of nitrocellulose, and one which is more suitable as a gunpowder. This product is translucent, tough, and leathery and in use practically smokeless; but the essential characteristic features of the product obtained by proportioning the trinitro and dinitro constituents of the explosive consist in that it burns at such a rate and yields such a volume of gases

that together give sufficient velocity to the projectile without giving rise to dangerous or excessive pressures within the firearm, rendering the use of the explosive perfectly safe, 55 a desideratum that has long been sought, and is still the great difficulty manufacturers have to contend with. Moreover, by proportioning the nitro constituents as described there is no exudation of nitroglycerin, as is the case 60 with many of this class of explosives, and particularly with the smokeless explosives manufactured by the Abel process.

The following weight proportions form suitable compounds:

|                                 | Per cent. | Per cent. |
|---------------------------------|-----------|-----------|
| Insoluble nitrated cotton ..... | 40        | 47        |
| Soluble nitrated cotton.....    | 20        | 23        |
| Nitroglycerin .....             | 40        | 30        |
|                                 | 100       | 100       |

The amount of acetone necessary for dissolving the insoluble nitrated cotton would be in the first case about thirty parts and in the second about forty.

As is well known in the manufacture of nitrocellulose compounds with nitroglycerin, it is of comparatively small importance, except for practical convenience, whether the solvent is first added to guncotton (trinitrocellulose) for dissolving it and then combining the solution with colloidion-cotton (dinitrocellulose) and nitroglycerin, the two latter ingredients being already combined or not, or whether the solvent is first added to the nitroglycerin and then the guncotton and then the collodion-cotton added, or whether the compound or mixture of the highly-nitrated and of the less highly-nitrated cellulose is first treated with the solvent and then mixed with the nitroglycerin. In all cases, as is well known, the nitroglycerin is only able to dissolve the dinitrocellulose, while the acetone or acetic ether dissolves the trinitrocellulose.

The manufacture is by preference carried on at the ordinary temperature. The gelatinous mass resulting from a sufficient kneading of the compound may then be granulated by the usual means. The solvent having evaporated or been otherwise removed by known means, the material is ready for use.

With the ingredients named may also be incorporated suitable material in small proportions for modifying the explosiveness and for protecting against atmospheric influences, such as paraffin, shellac, or graphite, all of which are well known for such purposes.

I claim—

1. In the manufacture of substantially smokeless explosives a base consisting of two parts of trinitrocellulose and one part of dinitrocellulose, substantially as and for the purposes set forth.

2. A substantially smokeless explosive consisting of trinitrocellulose, dinitrocellulose and nitroglycerin in the proportions substantially as herein described, said explosive being tough, leathery, and translucent, and characterized by its combined qualities as to rate of combustion, yield of gases, non-exudation of the nitroglycerin, and its constancy.

GEORGE GUILLAUME ANDRÉ.

Witnesses:

GEO. J. B. FRANKLIN,  
WALTER J. SKERTEN,